# EUROPEAN PATENT SPECIFICATION

(11) **EP 0 049 052 B1**
(45) Date of publication and mention of the grant of the patent: **06.02.1985**
(21) Application number: 81303978.1
(22) Date of filing: 01.09.1981
(51) Int. Cl.: D02G 1/12

(54) **Yarn crimping by means of a stuffer-box**
Kräuseln von Garnen mittels einer Stauchkammer
Frisage de fils au moyen d'une boîte de bourrage

(30) Priority: 04.09.1980 GB 8028504
(43) Date of publication of application: 07.04.1982
(73) Proprietor: PLASTICISERS LIMITED, Bradford, BD11 1BY Yorkshire (GB)
(72) Inventor: Firth, Colin, Drighlington Bradford (GB)
(74) Representative: Stringer, David Hiram

## Description

The present invention relates to apparatus and a method for use in the texturising of single or multi-filament yarn.

In particular the present invention relates to the texturising of yarn manufactured from a thermoplastic material.

Yarn manufactured from a thermoplastic material can be texturised to bulk the yarn, in a number of known ways. However, the bulking of the yarn is usually only in a two-dimensional plane e.g. the yarn takes on a saw-tooth configuration. Thus the yarn does not necessarily provide a uniform bulking, i.e. texturising in all possible directions transverse to the yarn.

Texturising in three dimensions is possible using the apparatus disclosed in U.S. Patent Specification US-A-3 482 294 (Joly). This apparatus has a stuffer chamber formed by a rigid coiled spring which is supported only at one end, the spring having a uniform diameter throughout. Filaments can be collected and bulked in the coiled spring and ejected as friction between bulked filament and spring coils is overcome by the feed pressure.

The aim of the present invention is to provide a further method and apparatus for producing a yarn which is more aesthetically pleasing than prior art 2-dimensional yarns as referred to hereabove, the method and apparatus being less capital intensive than previous arrangements.

According to the present invention there is provided texturising apparatus for use in providing a three-dimensionally-bulked yarn, comprising a coiled spring which is secured at one end and which forms a stuffer chamber to which one or more filaments of a thermoplastics material can be continuously fed, characterised in that the coiled spring is tapered, fixedly secured at each end thereof, and maintained in a loaded condition, the spring being widest at its outlet end.

The apparatus of the present invention utilises a transporter for the continuous filament or filaments, which connects with the narrow end of the spring, the spring being preferably tensioned between its ends. Alternatively the spring may be an open wound spring which is compressed. The transporter preferably utilises a stream of gaseous fluid to carry the filament or filaments continuously forward into the stuffer chamber formed by the tapered spring. The gaseous fluid is preferably air which is preferably dry and fed at a desired substantially constant speed. The temperature of the air should be adjusted to supply the requisite additional heat required for setting the filament or filaments, the filaments having been preheated before reaching the stuffer chamber.

In use the filament or bundle of filaments is fed into the narrow end of the coiled spring forming the stuffer chamber, the filament or filaments being folded within the chamber due to their rate of feed e.g. 1000 m/min, and forming a plug of filament at the outlet end of the spring, the temperature of the filament being sufficient to allow the filaments to set in the folded position. The folding of the filament is randomly in all directions transverse to the axis of the spring so that a three-dimensional bulking of the filament is achieved. In the event that the plug does not initially form, the wider outlet end of the spring may be blocked off at slow speeds, for a short period of time to prevent the egress of yarn and cause the plug to form.

The initially formed plug will continue to grow and extend back towards the inlet end of the spring. As the plug grows so it covers the gaps between adjacent coils of the spring reducing the area through which the air from the transporter can escape. Thus the air pressure on the plug increases tensioning and stretching the inlet end of the spring further and simultaneously closing the coils together at the outlet end so as to reduce the frictional grip of the spring coils, until the air pressure is able to overcome the frictional grip of the spring coils on the plug and the bulked filaments are forced out of the spring. At this point the area through which transporter air can escape is increased so that the pressure on the plug decreases allowing the spring to contract. The process continues the plug being continuously formed, so that the bulked yarn is ejected continually, the spring oscillating back and forth. This is a continuous operation with the bulked yarn merely being collected from the outlet of the stuffer chamber, it being unnecessary to draw the yarn therefrom.

The maximum possible speed of operation is determined by the taper of the spring, speeds of several thousand metres/minute being possible. However, a speed of 1000 metres/minute is preferably required with a minimum of 600 metres/minute.

For the yarn to be forced from the stuffer chamber the frictional grip of the spring on the plug is important and this can be rendered substantially constant for different filaments e.g. for different colours of filament wherein the pigment can alter the surface friction characteristic, by the addition of a fibre lubricating agent e.g. Limanol P81 a proprietary product manufactured by Schill Scheillacher. The use of such fibre lubricating agent provides for substantially uniform bulking of the yarns, this being clearly desirable.

if the speed and/or friction of the spring/fila- ment interface, are too great then the plug within the spring will increase in size and back into the transporter blocking further operation. The taper and other characteristics of the spring are therefore important for the continuous operation of the apparatus as desired. The precise action of the spring is dependent upon the taper, the diameter of the wire or other material forming the spring, its length and pitch. Variation in these parameters will produce a variation of the effect of the spring on the filaments and they should be so chosen as to produce the optimum action on the filaments.

The filament or filaments may have any desired cross-section. Thus in addition to being round, the cross-section may be delta-shaped, rectangular, triangular or polynodal or may have three or more branches forming for example an X or Y configuration. Furthermore, when more than one filament is present in the yarn, filaments of different cross-sections may be used. The filaments may also be hollow.

The continuous filament or filaments may be composed of any thermoplastic synthetic plastics material capable of being formed into a foldable filament and filaments of different synthetic plastics materials may be present in the yarn. Preferably the synthetic thermoplastic material is a homopolymer or copolymer of polypropylene.

According to a further feature of the present invention there is provided a method of texturising yarn formed from one or more filaments of a thermoplastics material, said method comprising the steps of feeding one or more continuous filaments into the stuffer chamber formed by the tapered, coiled spring, which is maintained in a loaded condition, the chamber being maintained at an elevated temperature, and continuously folding said filament or filaments within said chamber whereby to fill at least a portion of the length of the chamber, maintaining said folded filament or filaments within said chamber for a period of time and at a temperature which sets the filament or filaments in the folded state, and allowing the yarn to spill out of the wider end of the tapered spring.

The present invention will now be further described, by way of example, with reference to the accompanying drawing in which one embodiment of the apparatus of the present invention is shown in partially cutaway perspective.

Referring to the drawing the transporter 1 is constructed of a hollow cylindrical body 3 through which a filament inlet pipe 5 extends, one end of pipe 5 connecting with a hole 7 in circular flange 9 of texturiser 11. Within body 3 which is sealed at each end to inlet pipe 5 are three angled air nozzle pipes 13 which connect with the interior of pipe 5. Thus by feeding heated air into body 3 via inlet 15, the air is passed via nozzle pipes 13 into pipe 5, the angled air jets thus formed, drawing the or each filament along inlet pipe 5 towards texturiser 11.

The texturiser 11 basically comprises two circular flanges 9 and 17, coaxially secured together by support rod 19. A tapered spring 21 is tensioned between flanges 9 and 17 and communicates with holes 7 and 23 in flanges 9 and 17 respectively. The tapered spring has its narrower end secured to flange 9 around inlet hole 7. Alternatively an open wound spring can be substituted for tensioned spring 21, the open wound spring being loaded under compression between flanges 9 and 17.

In use a filament or bundle of filaments is fed from a spool or spools (not shown) mounted on a creel if desired, through appropriate nip or guide rollers (not shown) both to maintain the desired rate of feed and to control the infeed tension of the filaments. Alternatively one or more bobbins of orientated yarns could serve as the feedstock, or the apparatus could draw the yarn or yarns into the texturiser. Various yarns e.g. different material and/or colour, could be fed simultaneously to the texturiser.

The filament or bundle of filaments is drawn through the transporter 1 by the air jets from nozzle pipes 13 and is fed into a stuffer chamber of texturiser 11, which is defined by tensioned tapered spring 21. The filament or filaments are preheated and the air drawing the filaments through the transporter is also at an elevated temperature which is sufficient to supply requisite heat for just setting the filaments. The filaments, due to their speed, fold across the inside of the spring in randomly orientated transverse directions and form a plug of filament. The filaments are thus compressed and heat set in the folded position. If the speed of the filaments is not sufficient to initially form the plug, the outlet of the texturiser can be closed off for an initial period of time to prevent the egress of yarn and allow the plug to form. Once started, the plug continues to extend backwards along the spring covering the interstices between the coils as it goes and thus restricting the area of the interstices through which the air from transporter 1 can escape. This increases the pressure on the plug and stretches the narrower inlet end of spring 21, and when this pressure reaches the level of the frictional forces holding the plug in place in the spring, part of the plug is ejected as bulked yarn, from the spring 21. This increases the total area between the coils of the spring through which air from the transporter 1 can escape, reduces the pressure on the plug and allows the spring to contract-the spring stretching again as the plug is formed. The spring thus oscillates back and forth as the plug is continuously formed and ejected. The diameter of the spring also oscillates as the plug is formed and ejected. Bulked yarn is thus continuously ejected from the spring and is preferably collected via a relaxation roller which allows the filament to cool sufficiently to set the crimp so that subsequent winding tension does not pull the crimp out. The relaxation roller also acts as a reservoir to allow compensation for tension control. Due to the folding of the filaments in randomly orientated directions transverse to the longitudinal axis of spring 21, a three-dimensional bulking of the filaments is achieved.

A plug of filaments thus remains at all times in the spring, an equilibrium being set up between the air pressure build up on the one hand, and the frictional forces between the spring coils and the plug. Critical parameters in this operation to produce desired output speeds for the bulked yarn of 1000 metres/minute with a minimum of 600 metres/minute, are the degree of taper of the spring i.e. the difference between the diameter of the spring ends relative to the spring length, the nature of the spring surface, the material of the spring and the filament material.

Having selected the above parameters to provide a given performance with a particular filament material, the bulking of that filament material and thus the performance of the apparatus, can be affected by changes in the nature of the filament. For example the addition of different pigments to the same basic filament material can result in different bulking, the surface friction coefficients changing due to the addition of pigment. Such variations can be minimised to produce substantially constant bulking by the use of a fibre lubricant e.g. Linamol P811 manufactured by Schill Scheillacher.

The invention will be further illustrated with reference to the following example:-

### Example 1

The procedure described above was carried out using a tow of polypropylene filaments and a transporter as illustrated in the drawing, with an air temperature of 165°C and at a pressure of 154 p.s.i. The tow has 120 filaments and the polypropylene had an m.f.i. of 10 and a denier per filament of 16.6. The dimensions of the tapered spring forming the texturiser were as follows:-

Spring diameter tapers uniformly during its length from 0.1875" to 0.25". (4.76 mm to 6.35 mm).

The product produced was a bulked yarn, the denier of which had increased over 20%, the bulking being three-dimensional.

## Claims

1. A texturising apparatus for use in producing a three-dimensionally bulked yarn, comprising a coiled spring which is secured at one end and which forms a stuffer chamber (21) to which one or more filaments of a thermoplastics material can be continually fed, characterised in that the coiled spring (21) is tapered, fixedly secured at each end thereof, and maintained in a loaded condition, the spring (21) being widest at its outlet end (23). 2. Apparatus as claimed in claim 1, characterised in that the spring (21) is tensioned between its ends.

3. Apparatus as claimed in claim 1, characterised in that the spring (21) is an open wound spring which is compressed.

4. Apparatus as claimed in any one of claims 1 to 3, characterised in that the tapered spring (21) is fixed between two planar flanges (9, 17) which are arranged parallel to each other, support rods (19) interconnecting said flanges (9, 17) and maintaining the flanges (9, 17) in spaced apart relationship, the ends of the spring (21) being secured to said flanges (9, 17) over coaxially aligned apertures (7, 23) in said flanges (9, 17).

5. Apparatus as claimed in any one of the preceding claims, characterised in that the narrower end (7) of the tapered spring (21) forming the stuffer chamber, is connected to a transporter (1) for the continuous filament or filaments.

6. Apparatus as claimed in claim 5, characterised in that the transporter (1) utilises a stream of gaseous fluid to carry the filament or filaments continuously forward.

7. Apparatus as claimed in claim 6, character used in that the gaseous fluid is dry air fed at a desired substantially constant speed.

8. A method of texturising yarn formed from one or more filaments of a thermoplastic material, using the apparatus of claim 1, characterised by the steps of feeding one or more continuous filaments into the stuffer chamber formed by the tapered, coiled spring (21), which is maintained in a loaded condition, the chamber being maintained at an elevated temperature, and continuously folding said filament or filaments within said chamber whereby to fill at least a portion of the length of the chamber, maintaining said folded filament or filaments within said chamber for a period of time and at a temperature which sets the filament or filaments in the folded state, and allowing the yarn to spill out of the wider end (23) of the tapered spring (21 ).

9. A method as claimed in claim 8, characterised in that the filament or filaments are treated with a lubricating agent before being fed to the stuffer chamber (21 ).

10. A method as claimed in claim 8 or 9, characterised in that the filament or filaments are fed to the stuffer chamber (21) by a flow of gaseous fluid.

11. A method as claimed in claim 10, characterised in that the gaseous fluid is dry air which is fed at a substantially constant speed, the temperature of the air being sufficient to supply the requisite additional heat required to set the filament or filaments, the filaments having been preheated before reaching the stuffer chamber (21

12. A method as claimed in any one of claims 8 to 11, characterised in that the filament or filaments are fed to the stuffer chamber (21) at 1000 metres/min.

## Patentansprüche

1. Texturiervorrichtung zum Herstellen eines dreidimensional gekräuselten Garns mit einer Schraubenfeder, die an einem Ende befestigt ist und eine Stauchkammer (21) bildet, der ein oder mehrere Faden bzw. Fäden eines thermoplastischen Kunststoffmaterials kontinuierlich zugeführt werden kann bzw. können, dadurch gekennzeichnet, daß die Schraubenfeder (21) konisch ausgebildet, an beiden Enden fest angebracht und in beladenem Zustand gehalten wird, wobei die Feder (21) ihre breiteste Abmessung an ihrem Austrittsende (23) aufweist.

2. Vorrichtung nach Anspruch 1, dadurch gekennzeichnet, daß die Feder (21) zwischen ihren Enden vorgespannt ist.

3. Vorrichtung nach Anspruch 1, dadurch gekennzeichnet, daß die Feder (21) eine offen gewickelte, uner Druckbeanspruchung stehende Feder ist.

4. Vorrichtung nach einem der vorhergehenden Ansprüche 1 bis 3, dadurch gekennzeichnet, daß die konische Feder (21) zwischen zwei ebenen Flanschen (19, 17) befestigt ist, die zueinander parallel angeordnet und durch Stützstangen (19) miteinander verbunden und in einem Abstand voneinander gehalten sind, wobei die Enden der Feder (21) an diesen Flanschen (19, 17) über in letzteren koaxial zueinander ausgerichteten Durchbrechungen (7, 23) befestigt sind.

5. Vorrichtung nach einem der vorhergehenden Ansprüche, dadurch gekennzeichnet, daß das engere Ende (7) der die Stauchkammer bildenden konischen Feder (21) mit einer Transporteinrichtung (1) für den kontinuierlichen Faden bzw. die kontinuierlichen Fäden verbunden ist.

6. Vorrichtung nach Anspruch 5, dadurch gekennzeichnet, daß die Transporteinrichtung (1) einen Strom eines gasförmigen Fluids verwendet, um den Faden oder die Fäden kontinuierlich vorwärtszutragen.

7. Vorrichtung nach Anspruch 6, dadurch gekennzeichnet, daß das gasförmige Fluid trockene Luft ist, die mit einer gewünschten im wesentlichen konstanten Geschwindigkeit zugeführt wird.

8. Verfahren zum Texturieren von Garn, das aus einem oder mehreren Faden bzw. Faden aus thermoplastischem Material gebildet ist unter Verwendung der Vorrichtung gemäß Anspruch 1, gekennzeichnet durch die Schritte des Einführens von einem kontinuierlichen Faden oder mehreren kontinuierlichen Fäden in die von der konischen Schraubenfeder (21) gebildeten Stauchkammer, die in beladenem Zustand und unter erhöhter Temperatur gehalten wird, und des kontinuierlichen Faltens des Fadens bzw. der Fäden innerhalb der Kammer, um dadurch zumindest einen Teil der Länge der Kammer zu füllen, wobei der gefaltete Faden oder die gefalteten Fäden innerhalb der Kammer für eine Zeitspanne in der Kammer auf einer Temperature gehalten werden mit dem Ergebnis, daß Faden oder Fäden in gefaltetem Zustand fixiert werden, wobei das Garn die Möglichkeit hat, aus dem breiteren Ende (23) der konischen Feder (21) auszutreten.

9. Verfahren nach Anspruch 8, dadurch gekennzeichnet, daß Faden oder Fäden mit einem Schmiermittel versehen werden, bevor sie die Stauchkammer (21) zugeführt werden.

10. Verfahren nach Anspruch 8 oder 9, dadurch gekennzeichnet, daß Faden oder Fäden durch einen Strom eines gasförmigen Fluids der Stauchkammer (21) zugeführt werden.

11. Verfahren nach Anspruch 10, dadurch gekennzeichnet, daß das gasförmige Fluid trockene Luft ist, die mit im wesentlichen konstanter Geschwindigkeit zugeführt wird und die Temperatur der Luft ausreicht, um die zusätzliche Hitze zuzuführen, die erforderlich ist, um Faden oder Faden zu fixieren, wobei die Fäden vor Erreichen der Stauchkammer (21) vorerhitzt worden sind.

12. Verfahren nach einem der Ansprüche 8 und 11, dadurch gekennzeichnet, daß Faden oder Fäden der Stauchkammer (21) mit 1000 m/min. zugeführt werden.

## Revendications

1. Appareil de texturation destiné à être utilisé pour la production d'un fil gonflé de façon tri-dimensionnelle, comprenant un ressort à boudin qui est fixé à une extrémité et qui forme une chambre de bourrage (21) dans laquelle on peut introduire en continu un ou plusieurs filaments d'un matériau thermoplastique, caractérisé par le fait que le ressort à boudin (21) est conique, qu'il est attaché de façon à chacune de ses extrémités, et qu'il est maintenu dans un état de charge, le ressort (21) étant plus large à son extrémité de sortie (23).

2. Appareil selon la revendication 1, caractérisé par le fait que le ressort (21) est tendu entre ses extrémités.

3. Appareil selon la revendication 1, caractérisé par le fait que le ressort (21) est un ressort enroulé ouvert, qui est comprimé.

4. Appareil selon l'une quelconque des revendications 1 à 3, caractérisé par le fait que le ressort conique (21) est fixé entre deux flasques plans (9, 17) qui sont parallèles entre eux, des tiges support (19) raccordant entre eux lesdits flasques (9, 17) et maintenant un desdits flasques (9, 17) écartés l'un de l'autre, les extrémités du ressort (21) étant fixées auxdits flasques (9, 17) sur des ouvertures (7, 23) ménagées de façon coaxiale dans lesdits flasques (9, 17).

5. Appareil. selon l'une quelconque des revendications 1 à 4, caractérisé par le fait que l'extrémité étroite (7) du ressort conique (21) formant le chambre de bourrage est raccordée à un transporteur (1) du ou des filament(s) continu(s).

6. Appareil selon la revendication 5, caractérisé par le fait que le transporteur (1) utilise un courant de fluide gazeux pour véhiculer le filament ou les filaments vers l'avant et de façon continue.

7. Appareil selon la revendication 6, caractérisé par le fait que le fluide gazeux est de l'air sec fourni à une vitesse souhaitée sensiblement constante.

8. Méthode pour texturer un fil formé d'un ou de plusieurs filaments constitués d'un matériau thermoplastique, utilisant l'appareil de la revendication 1, caractérisée par les étapes consistant à introduire un ou plusieurs filaments à l'intérieur de la chambre de bourrage formée par le ressort à boudin conique (21 qui est maintenu dans un état de charge, la chambre étant maintenue à une température élevée et consistant à plier en continu le(s) filament(s) en question à l'intérieur de ladite chambre jusqu'à remplir au moins une portion de la longueur de la chambre, à maintenir le(s) dit filament(s) plié(s) à l'intérieur de ladite chambre pendant une période de temps et à une température qui fixe le filament ou les filaments dans l'état plié et consistant à permettre au fil de s'éjecter de l'extrémité large (23) du ressort conique (21).

9. Méthode selon la revendication 8, caractérisée par le fait que le ou les filaments sont traités avec un agent de lubrification avant d'être introduits dans la chambre de bourrage.

10. Méthode selon les revendications 8 ou 9, caractérisée par le fait que le ou les filaments sont introduits dans la chambre de bourrage par un flux de fluid gazeux.

11. Méthode selon la revendication 10, caractérisé par le fait que le fluide gazeux est de l'air sec qui est amené à une vitesse sensiblement constante, la température de l'air étant suffisante pour fournir le chaleur supplémentaire nécessaire pour fixer le ou les filaments, ces derniers ayant été pré-chauffés avant d'atteindre la chambre de bourrage (21).

12. Méthode selon l'une quelconque des revendications 8 à 11, caractérisée par le fait que le ou les filaments sont amenés à la chambre de bourrage (21) à une vitesse de 1000 mètres/minute.
